# EUROPEAN PATENT SPECIFICATION

(11) **EP 0 982 414 B1**
(45) Date of publication and mention of the grant of the patent: **28.04.2004**
(21) Application number: 98116225.8
(22) Date of filing: 27.08.1998
(51) Int. Cl.: D01D 5/24, D01D 5/253

(54) **Multilobal hollow filaments having stiffening ribs and stiffening webs**
Multilobale Hohlfilamente mit Versteifungsrippen und Versteifungszonen
Filaments creux multilobés ayant des nervures et des zones de raidissement

(43) Date of publication of application: 01.03.2000
(73) Proprietor: E.I. DU PONT DE NEMOURS AND COMPANY, Wilmington Delaware 19898 (US)
(72) Inventor: Bernaschek, Walter, 59269 Beckum (DE)
(74) Representative: KUHNEN & WACKER

(56) References cited:
- EP-A- 0 661 391
- US-A- 2 965 925
- US-A- 3 493 459
- US-A- 5 322 736

## Description

### BACKGROUND OF THE INVENTION

**Field of the Invention** The present invention relates to a multi-lobal hollow filament having stiffening ribs in the core portion and at least one transverse web in each lobe, and to a spinneret plate for producing the filament.

**Description of the Prior Art** Fibers useful for carpet manufacture exhibit certain desirable performance criteria. These criteria include good crush resistance, high cover and good soil hiding ability. The structure of the fiber is a determinative factor in the ability of a given fiber to meet these performance criteria.

The crush resistance of a carpet depends on the stability properties of the pile fibers used in the carpet. The higher the stability of the fiber, the more resistant to crushing is the carpet. The covering ability of a carpet is determined by the space occupied by the fiber cross-section. For a given crimp a measure of the space occupancy for a lobal fiber is given by the fiber's modification ratio. The higher the modification ratio of the fiber, the greater the covering ability of the carpet.

The presence of hollow regions in the interior of the fiber further increases the covering power and simultaneously increases its light scattering ability and decreases its luster. Thus, the presence of hollow regions coupled with the modification ratio, determine the fiber's covering and soil hiding ability. U. S. Patent 5,380,592 (Tung) and European Patent Office Publication 661,391 disclose a trilobal or tetralobal filament having a hollow core portion and an axially extending void in each lobe.

In another aspect hollow fibers with the same modification ratio and surface area as against solid fibers reduce the specific gravity according to the percentage of the fiber that is hollow. For example, a twenty percent hollow (or "void") ratio reduces the specific gravity or density for nylon fibers from 1.14 to 0.91 grams per cubic centimeter and reduces the specific gravity for polyester fibers from 1.35 to 1.08 grams per cubic centimeter (both twenty percent reductions). This is desirable for lightweight carpets, apparel or fabrics.

Designing the structure of the fiber to enhance one of these performance criteria is often detrimental to another performance criterion. For example, in U. S. Patent 5,208,107 (Yeh et al.), a multi-lobal synthetic fiber has a single axially extending central void. Although this structure may enhance the fiber's stability it is not well-suited to enhance the soil hiding ability of the fiber.

As another example, U. S. Patent 4,770,938 (Peterson et al.) shows a trilobal fiber having elongated voids extending through each lobe. Although such a structure increases the soil hiding capability of the fiber the lack of rigidity makes the lobes prone to collapse, thus detracting from the crush resistance of the fiber. If the structure of the lobes were rigidified as in U. S. Patent 5,322,736 (Boyle et al.) the fiber becomes more crush resistant, at the cost of increased polymer.

US-A-3,493,459 discloses a multi-lobal filament having a central axially extending hole and a smaller axially extending hole in each of the filament's lobes.

In view of the foregoing, it is believed advantageous to provide a multi-lobal fiber structure that optimizes the fiber's soil hiding and covering ability, without sacrificing crush resistance and without increasing the volume of the polymer material in the fiber.

Subject matter of the present invention is a thermoplastic filament according to claim 1.

Preferred embodiments thereof are subject matter of claims 2 to 6.

A further subject matter of the present invention is a spinneret plate according to claim 7 for producing a thermoplastic filament according to the present invention.

Preferred embodiments thereof are subject matter of claims 9 to 13.

A further subject matter is a carpet yarn according to claim 14 having at least one thermoplastic filament according to the present invention.

Still another subject matter is the use of a yarn according to the present invention for the manufacture of a carpet.

### SUMMARY OF THE INVENTION

The present invention is directed to a thermoplastic synthetic polymer filament comprising a core portion having a number N lobes joined thereto. Preferably, three or four lobes may be provided, thereby respectively defining trilobal and tetralobal filament configurations. Each lobe has a tip thereon and is joined to the core portion along an inscribing circle. The filament has a central axis extending therethrough. N stiffening ribs are formed in the core portion, with the ribs extending radially inwardly toward the axis of the filament. The stiffening ribs cooperate to define at least N hollow regions in the core portion. Each hollow region in the core aligns radially with a respective lobe.

In one embodiment the radially inner ends of the stiffening ribs may be spaced from each other and from the central axis of the filament, thereby to define passages within the core portion through which the hollow regions communicate with each other. Alternatively, each stiffening rib may extend to meet and join to the other of the ribs along the axis of the filament whereby the hollow regions in the core portion are isolated from each other. The ribs in the core portion form abutting members on the interior of the filament that contact with each other under high face loading to enhance the stiffness and load capacity of the filament.

Each lobe has at least one opening disposed between the tip of the lobe and the inscribing circle. The opening in each lobe and the hollow region of the core portion corresponding to that lobe cooperate to define a transverse stiffening web across each lobe. The presence of the transverse stiffening web across each lobe prevent the lobe lateral edges from being deformed towards the exterior of the filament, resulting in a high degree of rigidity and crush resistance.

In accordance with another modified embodiment each lobe may be provided with a second opening therein so that the first and the second openings cooperate to define a second transverse web extending across the lobe. When provided the second opening in each lobe is disposed between the first opening and the tip of the lobe.

In yet another embodiment the major portion of each lateral edge of each lobe may be substantially linear over substantially its entire length. The arm angle for linear edge filament lies in the range from about zero to about fifteen degrees. Alternatively, the major portion of each lateral edge is convexly curved over substantially its entire length.

Any filament in accordance with any of the various embodiments of the invention illustrated herein has a modification ratio that lies in the range from about 1.6 to about 4.0, and preferably in the range from about 2.0 to 3.0, and most preferably in the range from about 2.3 to about 2.6. The filaments have a total void percentage in the range from about seven (7%) to about thirty percent (30%), and more preferably, in the range from about twelve (12%) to about twenty-two percent (22%).

In another aspect the present invention is directed to a spinneret plate for producing any of the thermoplastic synthetic polymer filaments summarized above. The spinneret plate comprises a cluster of N pairs of peripheral slot segments centered about a central point. To form lobes having substantially linear or convexly curved lateral edges, the peripheral slot segments are either substantially linear or convexly curved, respectively.

Each peripheral slot segment in each pair is joined to an adjacent peripheral slot segment at a junction point. A rib-forming slot extends radially inwardly from each junction point toward the central point of the cluster. The distance between the junction point and the central point of the cluster occupied.by each rib-forming slot determines whether the ribs meet at the axis or whether the inner ends of the ribs are spaced from the axis.

Each slot segment in each pair is confrontationally disposed with respect to a slot segment in another pair. At least one web-forming slot extends from each peripheral slot segment toward the peripheral slot segment with which it is confrontationally disposed. If desired, a second web-forming slot may also extend from each peripheral slot segment toward the confrontationally disposed peripheral slot segment.

### BRIEF DESCRIPTION OF THE DRAWINGS

The invention will be more fully understood from the following detailed description, taken in connection with the accompanying drawings, which form a part of this application and in which:
Figure 1A is a cross section view of a straight-edged trilobal filament in accordance with the present invention in which each lobe has a single transverse stiffening web and a single opening therein and in which the hollow regions of the core portion communicate through constricted passages defined by the stiffening ribs;
Figure 1B is a bottom view of a spinneret plate in accordance with the present invention for producing the straight-edged trilobal filament of Figure 1A;
Figure 2A is a cross section view of a straight-edged trilobal filament generally similar to that shown in Figure 1A in which the stiffening ribs connect with each other to isolate the hollow regions defined in the core portion;
Figure 2B is a bottom view of a spinneret plate in accordance with the present invention for producing the trilobal filament of Figure 2A;
Figure 3A and Figure 4A are cross section views analogous to the views shown in Figures 1A and 2A, respectively, of straight-edged trilobal filaments in which each lobe has a second transverse stiffening web and a second opening therein;
Figure 3B and Figure 4B are bottom views of spinneret plates in accordance with the present invention for producing the trilobal filaments of Figures 3A and 4A, respectively;
Figure 5A, Figure 6A, Figure 7A and Figure 8A are each cross section views analogous to the view shown in Figures 1A through 4A, respectively, of trilobal filaments in which the lateral edges of each lobe are convexly curved;
Figure 5B through Figure 8B are bottom views of spinneret plates in accordance with the present invention for producing the trilobal filaments of Figures 5A through 8A, respectively;
Figure 9A and Figure 10A are cross section views analogous to the views shown in Figures 1A and 2A, respectively, of tetralobal filaments in which each lobe has straight-edges and a single opening therein;
Figure 9B and Figure 10B are bottom views of spinneret plates in accordance with the present invention for producing the tetralobal filaments of Figures 9A and 10A, respectively;
Figure 11A and Figure 12A are cross section views analogous to the views shown in Figures 5A and 6A, respectively, of tetralobal filaments in which each lobe has convexly curved edges and a single opening therein;
Figure 11B and Figure 12B are bottom views of spinneret plates in accordance with the present invention for producing the trilobal filaments of Figures 11A and 12A, respectively;
Figure 13A is a cross section view analogous to the view shown in Figure 3A showing a tetralobal filament in which each lobe has straight edges with two openings therein, and in which the hollow regions of the core portion communicate through constricted passages defined by the stiffening ribs;
Figure 13B is a bottom view of a spinneret plate in accordance with the present invention for producing the straight-edged tetralobal filament of Figure 13A;
Figure 14A is a cross section view analogous to the view shown in Figure 8A showing a tetralobal filament in which each lobe has convexly curved edges with two openings therein, and in which the stiffening ribs connect with each other to isolate the hollow regions defined in the core portion; and
Figure 14B is a bottom view of a spinneret plate in accordance with the present invention for producing the tetralobal filament having convexly curved edges as shown in Figure 14A.

### DETAILED DESCRIPTION OF THE INVENTION

Throughout the following detailed description similar reference numerals refer to similar elements in all Figures of the drawings.

**Filament** Figure 1A is a cross section view of a trilobal thermoplastic synthetic polymer filament generally indicated by the reference character 10 in accordance with the present invention. A filament in accordance with the present invention may be prepared using any synthetic, linear, thermoplastic melt-spinnable polymer, including polyamides, polyesters, and polyolefins. After melting the polymer is extruded ("spun") through a spinneret plate (to be described hereinafter) under conditions which vary depending upon the individual polymer and the particular filament being spun thereby to produce a filament having a desired denier and a desired void percentage. Void percentage can be increased by a more rapid quenching and increasing the melt viscosity, which can slow the flow allowing sturdy, pronounced molding to occur.

The filament 10 shown in Figure 1A has a central core portion 12 having three lobes 14A, 14B, and 14C joined thereto (i. e., the number N = three). An axis 10A extends centrally and axially through the core portion 12 of the filament 10. Each lobe 14A, 14B, 14C terminates in a generally rounded tip 16A, 16B, 16C, respectively.

The tips 16A, 16B, 16C of each lobe 14A, 14B, 14C lie on a circumscribing circle 18 having a radius R₁ centered on the axis 10A. The junction between each lobe 14A, 14B, 14C and the core portion 12 lies on an inscribing circle 22 having a radius R₂ centered on the axis 10A. The modification ratio (i. e., the ratio of the radius R₁ to the radius R₂) of the filament 10 is in the range from about 1.6 to about 4.0, more preferably in the range from about 2.0 to 3.0, and most preferably in the range from about 2.3 to about 2.6.

The major portion of each lateral edge 24A, 24B of each lobe 14A, 14B, 14C is substantially linear to impart a substantially "straight" appearance over substantially the entire length between the tip 16A, 16B, 16C and the joint of the respective lobe 14A, 14B 14C to the core portion 12. The lateral edges 24A, 24B of each lobe 14A, 14B, 14C converge toward each other to define an arm angle 26 for each lobe 14A, 14B, 14C. The arm angle 26 lies in the range from about zero to about fifteen (15°) degrees.

The core portion 12 has three stiffening ribs 30A, 30B, 30C formed therein. The ribs 30A, 30B, 30C lie within the inscribing circle 22 and extend within the core portion 12 in a radially inward direction toward the axis 10A of the filament. Each rib 30A, 30B, 30C has a respective inner end 32A, 32B, 32C thereon. The ribs 30A, 30B, 30C cooperate to define three hollow regions 36A, 36B, 36C in the core portion 12. The hollow regions 36A, 36B, 36C extend axially through the filament 10. Each hollow region 36A, 36B, 36C aligns in a radially (with respect to the central axis 10A) with a respective lobe 14A, 14B, 14C.

In accordance with the present invention each lobe 14A, 14B, 14C has at least one opening 40A, 40B, 40C, respectively, therein. The opening 40A, 40B, 40C in each respective lobe 14A, 14B, 14C is disposed between the lobe tip 16A, 16B, 16C and the inscribing circle 22. The openings 40A, 40B, 40C also extend axially through the filament 10. The opening 40A, 40B, 40C together with the hollow region 36A, 36B, 36C corresponding to the lobe cooperate to define a transverse stiffening web 42A, 42B, 42C extending across the lobe.

In the embodiment of the invention illustrated in Figure 1A the radially inner ends 32A, 32B, 32C of adjacent stiffening ribs 30A, 30B, 30C are spaced from each other and from the central axis 10A of the filament 10. The spacing between the inner ends 32A, 32B, 32C of adjacent ribs 30A, 30B, 30C defines passages 46A, 46B, 46C through which the hollow regions 36A, 36B, 36C may communicate with each other. In the embodiment illustrated the transverse dimension of the passages 46 is relatively constricted with respect to the transverse dimension of the associated hollow region 36, although such a relationship is not required.

In the embodiment shown in Figure 1A the hollow regions 36A, 36B, 36C and the passages 46A, 46B, 46C form a unitary void that extends centrally and axially through the core portion 12 of the filament 10. The relatively constricted shape of the passages 46A, 46B, 46C as compared to the hollow regions 36A, 36B, 36C imparts a generally "clover-like" or "propeller-like" shape to the unitary void.

The presence of the openings 40A, 40B, 40C together with the unitary central axial void formed by the hollow regions 36A, 36B, 36C and the passages 46A, 46B, 46C results in a filament 10 in which the cross section has a total void percentage (herein also "void%"; i. e., the percentage of "open space" on the interior of the filament) that lies in the range from about seven (7%) to about thirty percent (30%). More preferably, the total void percentage lies in the range from about twelve (12%) to about twenty-two percent (22%). As will be demonstrated by the Examples following herein the filament 10 in accordance with the present invention embodies various structural compromises that result in acceptable performance as measured against all desirable performance criteria. The modification ratio, arm angle and void percentage cooperate to impart high cover, low glitter and good soil hiding performance to the filament 10. The stiffening web 42 in each lobe 14 retards the collapse of the lobe due to high force loading, while the ribs 30A, 30B, 30C in the core portion 12 form abutting members on the interior of the filament that contact with each other under high face loading to enhance the stiffness and load capacity of the filament. The presence of these structural features imparts good crush resistance to the filament.

**Spinneret Plate** Figure 1B illustrates the bottom surface 50B of a portion of a spinneret plate 50 for producing the filament 10 depicted in Figure 1A. As is known in the art a spinneret plate 50 is a relatively massive member having an upper surface and the bottom surface 50B. The upper surface of the spinneret plate is provided with a recess (not shown) whereby connection of the plate 50 to a source of polymer may be effected. Depending upon the rheology of the polymer being used the lower margins of the recess may be inclined to facilitate flow of polymer from the supply to the spinneret plate.

A capillary arrangement generally indicated by the reference character 54 extends through the plate 50 from its recessed upper surface to the bottom surface 50B. As is seen in Figure 1B the capillary arrangement 54 is defined by a cluster of peripheral slots 56A, 56B, 56C centered about a central point 58. Each peripheral slot 56A, 56B, 56C itself comprises a pair of slot segments indicated generally by the characters 60, 62. Thus, the peripheral slot 56A includes paired slot segments 60A, 62A; the peripheral slot 56B includes paired slot segments 60B, 62B; while the peripheral slot 56C includes paired slot segments 60C, 62C.

Each slot segment 60 is joined to its paired slot segment 62 at a junction point 64. A rib-forming slot 66 extends from each junction point 64 toward the central point 58 of the cluster. Each slot segment 60, 62 includes a generally linear portion 60L, 62L extending from the junction point 64 toward a generally rounded free end 60R, 62R. This arrangement serves to form the lobes 14 having linear lateral edges with generally rounded tips. The radius of the rounded free ends 60R, 62R is centered on an origin 68. Adjacent rounded ends 60R, 62R are spaced by a gap 63.

Each slot segment 60, 62 in a peripheral slot 56A, 56B, 56C is confrontationally disposed with respect to a slot segment forming another peripheral slot. Thus, in Figure 1B, the slot segment 60A included in the peripheral slot 56A is confrontationally disposed with respect to the slot segment 62C included in the peripheral slot 56C. The slot segment 62A included in the peripheral slot 56A is confrontationally disposed with respect to the slot segment 60B in the peripheral slot 56B. Similarly, the slot segment 62B included in the peripheral slot 56B is confrontationally disposed with respect to the slot segment 60C included in the peripheral slot 56C.

The distance between the junction point 64 and the central point 58 of the cluster occupied by each rib-forming slot 66 determines whether the radially inner end 32A, 32B, 32C of respective stiffening ribs 30A, 30B, 30C are joined together or are spaced from each other and from the central axis 10A of the filament 10 (as in Figure 1A). In general, to insure that the inner ends of the ribs join along the axis (and thus serve to isolate the hollow regions in the core portion from each other), the rib-forming slots should extend at least two-thirds of the distance between the junction point and the central point of the cluster. On the other hand, if the rib-forming slots extend less than one-half of the distance between the junction point and the central point of the cluster, then the inner ends of the ribs are spaced from each other and from the axis. If the rib-forming slots extend at least one-half but less than two-thirds of the distance between the junction point and the central point of the cluster, then the viscosity determines whether the ribs will join together at the axis of the filament.

Web-forming slots 70, 72 are provided on each peripheral slot segment 60, 62, respectively. The web-forming slot 70, 72 on any given slot segment 60, 62 extends toward a corresponding web-forming slot 70, 72 (as the case may be) provided on the slot segment 60, 62 with which the given slot segment is confrontationally disposed. The inside ends of the web-forming slots 70, 72 are separated by a space 74.

On Figure 1B (and on all of the other views of spinneret plates discussed herein) alphabetic reference characters are used to indicate the dimensions of various features of the spinneret plate 50 that form congruent features of the filament 10 of Figure 1A. In Figure 1B the character A refers to the distance from the center 58 of the cluster to the origin 68 of the rounded free ends 60R, 62R of the segments 60, 62, while the character B is the dimension of the radius of these free ends 60R, 62R. The character C represents the distance from the central point 58 to the inner wall of each slot 70, 72. The character D represents the spacing between the inner ends of the slots 66. The character E represents the dimension of the gap 63, while the character F represents the dimension of the space 74. The character G represents the width of the peripheral slots 56. The character H denotes the width of the slots 66, 72.

Polymer extruded from the capillary arrangement 54 forms the filament illustrated in Figure 1A. The presence of the generally linear portions 60L, 62L with generally rounded free ends 60R, 62R serves to form a filament 10 having lobes 14 with linear ("straight") lateral edges 24 and generally rounded tips 16. The spacing between the confronting inner ends of the web-forming slots 70, 72 insures that the polymer merges to complete a web 42 traversing each lobe 14.

Polymer emerging from the slots 66 defines the ribs 32. In Figure 1B, the rib-forming slots 66 occupy less than one-half of the distance between the junction point 64 and the central point 58 of the cluster, and the inner ends 32 of the stiffening ribs 30 are spaced from each other and from the axis and the hollow regions 36 communicate through the passages 46.

Typical numerical values of the various dimensions indicated by the alphabetic reference characters on Figure 1B are as follows (1 inch (") = 2.54 cm):
A = 0.033", B = 0.013", C = 0.021", D = 0.095",
E = 0.0038", F = 0.0040", G = 0.0022", and H = 0.0018".
These dimensions are given all at an arm angle of zero degrees.

Each of the spinneret plates 50 shown herein may be fabricated using the laser technique disclosed in U. S. Patent 5,168,143, (Kobsa et al., QP-4171-A), assigned to the assignee of the present invention.

A modified embodiment of the filament 10 is shown in Figure 2A. The modified filament 10 of Figure 2A is identical with that of Figure 1A in that it exhibits straight lobes with rounded lobe ends. However, the modified filament 10 of Figure 2A differs from the filament of Figure 1A in that the hollow regions 36 in the core portion 12 are totally isolated from each other. As is the case with the filament of Figure 1A the ribs 30 in the core and the stiffening web 42 in each lobe 14 places sufficient material between the hollow regions 36 and the openings 40 to retard crushing of the filament in case of high face loading.

Typical numerical values of the various dimensions indicated by the alphabetic reference characters on Figure 2B (at an arm angle of zero degrees) are as follows (1 inch (") = 2.54 cm):
A = 0.033", B = 0.013", C = 0.021, D = 0.066",
E = 0.0038", F = 0.0040", G = 0.0022", and H= 0.0018".

Particular attention is invited to the magnitude of the dimension D, the distance between the rib forming slots 66 and the center of the cluster 58. In Figure 1B the dimension D 0.24cm (0.095") is greater than the dimension D in Figure 2B 0.168 cm (0.066"). The rib-forming slots 66 in the spinneret of Figure 2B extend toward the central point 58 for a distance greater than two-thirds the distance between the junction point 64 and the central point 58 of the cluster. As a result the stiffening ribs 30 of the filament of Figure 2A join together to isolate the hollow regions 36 from each other. In Figure 1B the rib-forming slots 66 extend less than one-half the distance between the junction point 64 and the central point 58 of the cluster, so that the ends of the ribs 30 in Figure 1A are spaced from each other.

Figures 3A and 4A show still other modified embodiments of a filament 10 having straight lobes with rounded ends shown as in Figures 1A and 2A. However, the filament of Figure 3A and Figure 4A differs from its respective counterparts in Figure 1A and Figure 2A by the presence of a second opening 41 in each lobe 14. The second opening 41 is disposed between the first opening 40 and the tip 16 of the lobe 14. In each lobe the first opening 40 and the second opening 41 cooperate to define a second transverse stiffening web 43. The filament of Figures 3A and 4A each have sufficient material between the hollow regions 36 and the openings 40 to retard crushing of the filament in case of high face loading.

Figures 3B and 4B show spinnerets 50 used to produce the congruent filaments illustrated in Figures 3A, 4A, respectively. In Figures 3B and 4B each slot segment 60, 62, respectively, includes a second web-forming slot 71, 73. The second web-forming slot is located on a slot segment 60, 62 intermediate the first slot 70, 72 (as the case may be) and the free end 60R, 62R. The reference character C1 in these Figures 3B, 4B represents the distance from the central point 58 to the inner wall of each second web-forming slot 71, 73.

Typical numerical values of the various dimensions on Figure 3B (at an arm angle of zero degrees) are as follows (1 inch (") = 2.54 cm):
A = 0.047", B = 0.013", C = 0.038",
C1 = 0.021", D = 0.095", E = 0.0038",
F = 0.0040", G = 0.0022", and H = 0.0018"

For Figure 4B, typical numerical values of the various dimensions (at an arm angle of 0 degree) are (1 inch (")=2.54 cm):
A = 0.047", B = 0.013", C = 0.038",
C1 = 0.021", D = 0.066", E = 0.0038",
F = 0.0040", G = 0.0022", and H = 0.0018"

However, similar to the situation with the spinnerets of Figures 1B and 2B, the dimension D of the rib forming slot 66 is different in Figures 3B and 4B. In Figure 3B the dimension D = 0.24 cm (0.095"), (the slots 66 extend less than one-half the distance between the junction point 64 and the central point 58 of the cluster), thus forming a filament in which the ends of the ribs are spaced from each other (Figure 3A). In the spinneret of Figure 4B, the dimension D = 0.168 cm (0.066") (the slots 66 extend greater than two-thirds the distance between the junction point 64 and the central point 58 of the cluster), so that the inner ends of the ribs 30 contact each other (Figure 4A).

The filaments 10 shown in Figures 5A, 6A, 7A and 8A correspond those of Figures 1A and 4A, respectively, save for the configuration of the lobes 14. The filaments of Figures 5A, 6A, 7A and 8A each exhibit lobes 14 with convexly curved lateral edges 24 and nipple-shaped lobe ends 16. Each slot segment has rounded portions in the vicinity of the junction point 64 to define concave cusps 25 on the perimeter of the filament between adjacent lobes 14. In accordance with this invention all of these filaments have sufficient material between the lobes to avoid filament crushing under load.

The lobes 14 of the filaments of Figure 5A and Figure 6A each have a single stiffening rib 42. The core regions 36 in Figure 5A communicate with each other, while in Figure 6A the core regions 36 are isolated. The lobes 14 of the filaments of Figure 7A and Figure 8A each have a pair of stiffening ribs 42, 43. The core regions 36 in Figure 7A communicate with each other, while in Figure 8A the core regions 36 are isolated.

Figures 5B and 6B illustrate a spinneret structures corresponding to the filaments of Figures 5A and 6A. These spinneret structures are generally similar to those shown earlier except that the linear portions 60L, 62L present in the spinnerets of Figures 1B through 4B are omitted. Each slot segment 56 is defined by a rounded or arcuate portion 60R, 62R centered on an origin 68 that corresponds to each of the convexly curved lateral edges of the lobes. Each lobe 14 thus exhibits a configuration reminiscent of a gothic arch. The arcuate portions 60R, 62R are joined in the vicinity of the junction point 64 by a rounded transition region 65 that defines the concave cusps. The reference character A still denotes the distance from the center 58 of the cluster to the origin 68, while the reference characters B and B1 respectively denote the radius of the rounded portions 60R, 62R of the lobes and the radius of the transition region 65. Only one of each such radius is shown for clarity. The transverse dimension of the rib forming slot 66 is given by the character H, while the transverse dimension of the web forming slots 70, 72 is given by the character H1.

Typical numerical values of the various dimensions indicated by the alphabetic reference characters on both Figure 5B and Figure 6B are as follows (1 inch(")=2,54 cm):
A = 0.028", B = 0.040", B1 = 0.0085",
C = 0.020", E = 0.0038", F = 0.0040",
G = 0.0022", H = 0.0018", H1 = 0.0016",

In Figure 5A the hollow regions 36 communicate with each other through the passages 46 to impart "clover-like" shape to the unitary void in the core. In Figure 6A the hollow regions 36 are isolated from each other. As discussed in conjunction with Figures 2B and 4B, to form such filaments it is necessary merely to modify the distance that the rib-forming slots 66 extends toward the center 58, as denoted by the dimension D. In Figure 5B the dimension D is 0,025 cm (0.010") and the slots 66 occupy less than one-half the distance between the junction point 64 and the central point 58 of the cluster. In Figure 6B the dimension D = 0,017 cm (0.0066"), and the slots 66 occupy greater than two-thirds the distance between the junction point 64 and the central point 58 of the cluster.

Typical numerical values of the various dimensions indicated by the alphabetic reference characters on both Figure 7B and Figure 8B, are as follows (1 inch(")=2,54cm):
A = 0.048", B1 = 0.0085", C = 0.020", C1 = 0.039",
E = 0.0038", F = 0.0040", G = 0.0022",
H = 0.0018", H1 = 0.0016

In Figure 7B (your FIG.10A) the dimension D is 0.24 cm (0.095") and the slots 66 occupy less than one-half the distance between the junction point 64 and the central point 58 of the cluster, imparting a clover-like shape to the core region. In Figure 8B the corresponding dimension D is 0,017 cm (0.0066") and the slots 66 extend for greater than two-thirds the distance between the junction point 64 and the central point 58 of the cluster. The ribs 32 (Figure 8A) join each other.

Figures 1A through 8A illustrates the present invention as applied to a trilobal filament (i. e., the number N is three). However, the present invention may also be implemented in the form of a tetralobal filament (i. e., the number N is four) having four lobes 14A, 14B, 14C and 14D. The lobes may have either straight or convexly curved lateral edges, with either single or double stiffening webs in each lobe, and with either communal or isolated hollow regions in the core. Various embodiments of tetralobal filaments with a single opening in each lobe are shown in Figures 9A through 12A. Figures 13A and 14A illustrate tetralobal filaments having a pair of openings disposed in each lobe.

Figures 9A and Figure 10A show straight-edged tetralobal filaments with communicating and isolated hollow regions 36, analogous to the filaments of Figures 1A and 2A, respectively. Figure 11A and Figure 12A show tetralobal filaments in which each lobe has convexly curved edges, with either communicating or isolated hollow regions 36, analogous to the filaments of Figures 5A and 6A, respectively. In the filaments of Figures 11A and 12A, the convexly curved edges meet without the presence of the rounded cusp 25 (Figures 7A, 8A).

Figures 9B, 10B, 11B, 12B respectively show spinnerets for forming the filaments of Figures 9A, 10A, 11A, and 12A. Typical dimensions of the spinneret apertures of Figures 9B and 10B are respectively the same as those for the spinnerets of Figures 1B and 2B. The dimensions of the spinneret apertures for Figure 11B and Figure 12B are respectively the same as the dimensions of the spinnerets of Figure 5B and Figure 6B.

Figure 13A illustrates a straight-edged tetralobal filament produced using a spinneret such as that shown in Figure 13B. The filament has a pair of openings 40, 41 and a pair of webs 42, 43 in each lobe 14 and communicating hollow regions 36 in the core. Typical numerical values for the various features of the spinneret of Figure 13B would correspond to those of Figure 3B. To produce a straight-edged tetralobal filament with isolated hollow regions 36 in the core a spinneret sized and shaped analogously to that shown in Figure 4B may be used.

Figure 14A illustrates a tetralobal filament having convexly curved lateral edges. The filament has a pair of openings 40 in each lobe 14 and isolated hollow regions 36 in the core. Figure 14B illustrates a spinneret which may be used to produce this filament. Typical numerical values for the various features of the spinneret of Figure 14B would correspond to those of Figure 8B. A spinneret sized and shaped analogously to that shown in Figure 7B may be used to produce a convexly curved tetralobal filament with communicating hollow regions 36 in the core.

### TESTING METHODS

**Luster & Glitter--Yarn:** Luster is a property related to the reflection or refraction of parallel or directional light by various interfaces of the fiber. Lower luster corresponds to higher light scattering. Glitter is the property produced when light is reflected or refracted from an area of a fiber which distinguishes that area from its surroundings. It is usually described as a "sparkling" of the fiber. Lower glitter results in a fiber having a luster more like the luster of natural fiber.

The luster and glitter measurements set forth herein (Table 1) for the Comparative and the Example (inventive) yarn samples were obtained from reflectance readings made using a conventional photogoniometer-based luster measurement instrument. A fixed angle of incidence (45 degree) and varied angle of detection were used. Each yarn sample was wound in parallel on a 20 mm x 100 mm card and its reflectance measured by the instrument. The half-peak width (HPW) obtained from the recording chart of the instrument is a measure of luster, with a smaller HPW indicating higher luster. The results of this test are listed in Table 1 under the heading "HPW".

The luster and glitter of the Example and Comparative yarn samples were also determined using a subjective visual luster and glitter tests. The samples were irradiated using a high intensity light and viewed by six observers. The yarn sample with highest luster was rated with "5" and the yarn sample with lowest luster rated "1" by each observer. The rating for highest luster therefore was 6 x 5 = 30. These ratings are indicated in Table 1 under the heading "Subjective Luster". For glitter a ranking was used, i. e. highest glitter = "1", and lowest glitter = "5". These ratings are indicated in Table 1 under the heading "Glitter".

**Luster & Glitter-- Carpet:** The luster and glitter measurements set forth herein for carpet samples were obtained from internal reflection readings. The percentage of internal reflection or degree of light scattering inside the fiber is a measure for classifying luster, glitter, and soil hiding. The lower the luster, the lower the glitter and the better the soil hiding capability of the carpet. The "glycol test" was used for measuring the internal reflection of carpet yarns. The reflection from a standard velour, winch dyed #2038A disperse gray, was measured before and after immersion in glycol. In the presence of glycol, reflection from the fiber surfaces is suppressed because of refractive index similarity between glycol and nylon 6,6. The relative reduction of reflection proved to be a reproducible and reliable measure for the percentage external reflection of yarns. The internal refection is calculated subtracting the external reflection from one hundred.

To obtain external reflection, a colorimeter Colorgloss, type of light C/10o is used. The CIE-L* is a numerical value for lightness of a sample from 0-100 (zero = black, 100 = white). L*1 - value: lightness of the sample measured w/o glycol. L*2 - value: lightness of the sample measured in glycol.$\text{Percentage external reflection =} \frac{\text{L*1 - L*2}}{\text{L*1}} \text{x 100}$

The results of this test are reported in Table 2 under the heading "Internal Reflection".

Glitter of two Test Example samples and two Comparative carpet samples which were both irradiated by a high intensity light was also determined subjective-visually. A ranking system highest glitter = "1", and lowest glitter = "4" was used. The results of this test are reported in Table 2 under the heading "Glitter".

**Carpet Cover** Cover was determined subjectively by ranking the light transmittance through the carpet samples having only a primary backing. The lower the light transmittance the higher the cover or bulk in carpet. The results of this test are reported in Table 2 under the heading "Cover".

**Carpet Soiling** Carpet soiling was measured using the "Tetrapod" of four currently popular test methods. These test methods are: (1) Soil hiding-dry; (2) Soil hiding-wet; (3) Soil repellency-dry; and (4) Soil repellency-wet. The results of the carpet soiling properties are reported below in Table 3.

The Tetrapod tests consisted of a series of cylindrical drums each 20 cm. in diameter and 20 cm long. Each drum was rotated about the cylindrical axis on four rollers. Inside the drum was placed a four legged "walker" having rubber "soles" on the end of each leg. The "walker" has a hole in the center into which dirt was placed and was held in position by a sieve. The piece(s) of carpet (total area 19 cm x 62 cm) were held against the inside surface of the drum by metal clips. The "walker" was placed inside the drum and the whole rotated at 50 rpm. Over a period of about 10 minutes about three grams of soil fell through the sieve and was distributed evenly over the carpet.

Soil Hiding-Dry: This is the default "Tetrapod" Test and was the only soiling test in common use. Each 19cm x 62cm carpet sample was tested at a time. The tests lasted 3 hours and 20 minutes (10,000 turns). After this time all the soil has been ground into the carpet. Vacuuming does not alter the carpet appearance so it is usually omitted. Each carpet sample was compared visually against a control piece of carpet which has also been in the drum for 10,000 turns but without dirt. The comparison was done under standard lighting conditions using a gray scale [Deutsche Industrie Norm (hereafter "DIN") 54002].

Results from at least three independent observers were averaged to give a "note" from 1 (dirty) to 5 (clean). Half and quarter "notes" gradations are possible, defining a total of twenty-one possible different "notes".

Soil Hiding-Wet: The principle difference in this test was that the carpet was sprayed with 6 ml of water immediately before placing in the drum. The carpet must be allowed to dry before visual comparison.

Soil Repellency-Dry: In the soil hiding tests the soil has no choice: it ends up in the carpet. The purpose of the soil repellency tests is to give the soil a choice: between one of two carpets, or the vacuum cleaner.

Two different carpet samples, each 31cm x 19cm, were placed in the drum. The test was run for 10 minutes (500 turns) by which time all the soil has left the reservoir and was on or in the carpet. The carpet was then vacuumed using a upright vacuum cleaner with rotating brush. The vacuum cleaner sold by Nilsfisk as "Nilfisk GS 21" was used. Each tested piece was then compared with an untested piece of the same carpet, using the "note" method described above.

Soil Repellency-Wet: This is similar to the dry test. Each piece of carpet was sprayed with three (3) ml of water immediately before testing. After testing, the samples are allowed to dry overnight before vacuuming.

**Carpet Wear** Carpet was measured using (1) the static loading test; (2) the Vetterman drum test; and (3) the Castor chair test.

Static Loading Static loading was measured according to DIN 54316 using a chair leg test to determine the compression behavior of a carpet sample loaded two hours at a pressure of 2.2 kg/cm². After a sixty minutes decompression time the remaining compression depth was measured. Original and final carpet pile height gives a rating based on a formula according to DIN 54316. The higher the rating number the better the performance.

Vetterman Drum Testing the change of the carpet appearance under mechanical loading was done by fixing the carpet sample inside metal drum with an internal diameter of seventy (70) cm according to DIN 54328. The drum was rotated 22,000 revolutions, with the direction of rotation reversed every five minutes. Throughout the rotation a 7.6 kg heavy round steel ball fitted with fourteen rubber studs rolled over the carpet. The judgment or classification of the carpet appearance change is done subjective-visually, with the higher the rating number the better the performance.

Castor Chair The suitability of a carpet for wear or loading by office roller chairs was tested by the Castor Chair according to DIN 54324. After 5000 and 25,000 turns a subjective-visual classification of the appearance change of the carpet pile takes place according to DIN 54328. The higher the rating number the better the performance of the carpet.

The results of the carpet wear properties are reported below in Table 4.

### EXAMPLES

Three embodiments of nylon 6,6 bulked continuous filament ("BCF") yarn in accordance with the present invention ("Test Examples") were produced and compared with two prior art nylon 6,6 bulked continuous filament yarns ("Comparative Examples") having a solid trilobal and a hollow, square cross-section, respectively. The nylon 6,6 polymer used for all of the yarns had a relative viscosity of 75-80 RV, and contained no delustering additives other than TiO₂. Identical process conditions for spinning, drawing, and bulking were used for all yarns.

The example yarns in accordance with the present invention were the following:
Test Example 1 A trilobal hollow filament yarn as illustrated in Figure 2A having sixty-four (64) filaments and 1360 dtex, produced using the spinneret of Figure 2B.
Test Example 2 A trilobal hollow filament yarn as illustrated in Figure 1A having sixty-four (64) filaments and 1360 dtex, produced using the spinneret of Figure 1B.
Test Example 3 A trilobal hollow filament yarn as illustrated in Figure 6A having sixty-four (64) filaments and 1360 dtex, produced using the spinneret of Figure 6B.

The comparison yarns were the following:
Comparison A A trilobal, solid filament yarn having sixty-eight (68) filaments and 1260 dtex such as the yarn sold by E. I. du Pont de Nemours and Company as DuPont 1301-O bright solid trilobal having a modification ratio of 2.6.
Comparison B A square hollow filament yarn having sixty-four (64) filaments and a linear density of 1360 dtex such as the yarn sold by E. I. du Pont de Nemours and Company as Du Pont 1401-D bright square four-hole cross-section having a percent hollow of 14.6 and a modification ratio of 1.4.

The optical properties of the yarns having a TiO₂ content of 0.02% (bright) were determined by the described methods for luster and glitter, and the results are reported below in Table 1.

**TABLE 1**

| Cand. | MR | Void% | HPW Luster | Subjective Luster | Glitter |
|---|---|---|---|---|---|
| Comp.A | 2.6 | 0 | 6.1 | 30 | 1 |
| Comp.B | 1.4 | 14.6 | 7.8 | 24 | 2 |
| Test Ex.1 | 2.6 | 14.3 | 9.3 | 12 | 4 |
| Test Ex.2 | 2.6 | 15.7 | 9.9 | 7 | 5 |
| Test Ex.3 | 2.6 | 11.5 | 9.0 | 17 | 3 |

Carpet: In order to illustrate the invention concerning optical-, cover/bulk-, mechanical-, and soiling-properties velour carpets of the BCF-yarns with following carpet constructions were made and tested: 68-77 stiches 1/10 Gauge (Fadenanzahl/38,1 mm) (1/10 inch gauge), 570 g/m2 pile weight, 6 mm pile height. Then #2038A disperse gray, latex and "ActionBac" backing for appearance retention, #9719 acid beige, latex for soiling.

The results of the optical and cover/bulk properties are reported below in Table 2.

**TABLE 2**

| Cand. | MR | Void% | Internal Reflection | Glitter 1= High | Cover 1= High |
|---|---|---|---|---|---|
| Comp.A | 2.6 | 0 | 10.4% | 1 | 4 |
| Comp.B | 1.4 | 14.6 | 53.0 | 2 | 3 |
| Test Ex.1 | 2.6 | 14.3 | 53.5 | 3 | 2 |
| Test Ex.2 | 2.6 | 15.7 | 58.5 | 4 | 1 |

**TABLE 3**

| | | | | -----Tetrapod Soiling----- | | | |
|---|---|---|---|---|---|---|---|
| Cand. | MR | Void% | TiO₂% | Dry | Dry/ Cleaned | Wet | Wet/ Cleaned |
| Comp.A | 2.6 | 0 | 0.02 | 3.50 | 3.75 | 1.50 | 2.25 |
| Comp.B | 1.4 | 14.6 | 0.02 | 3.50 | 4.00 | 2.25 | 3.00 |
| Test Ex.1 | 2.60 | 14.3 | 0.02 | 3.25 | 3.75 | 2.00 | 2.75 |
| Test Ex.2 | 2.60 | 15.7 | 0.02 | 3.50 | 4.00 | 1.75 | 2.50 |

**TABLE 4**

| Cand. | MR | Void% | TiO₂% | Static Loading | Vetterman Drum | Castor Chair |
|---|---|---|---|---|---|---|
| Comp.A | 2.6 | 0 | 0.02 | 3.6 | 2.0 | 2.3 |
| Comp.B | 1.4 | 14.6 | 0.02 | 3.6 | 2.5 | 2.6 |
| Test Ex.1 | 2.6 | 14.3 | 0.02 | 3.8 | 2.0 | 2.6 |
| Test Ex.2 | 2.6 | 15.7 | 0.02 | 3.5 | 2.0 | 2.4 |

### Results

The yarn and carpet results shown in Tables 1-4 reveals a significant glitter/luster reduction and improvement in cover of the invented hollow trilobal as against prior art solid trilobal and hollow square cross-section filament or fiber products. Carpet wear and soiling performance of the new hollow trilobal fibers are also better than solid trilobal fibers.

From the foregoing it may be appreciated that the present invention is directed to multi-lobal filaments that reflect light diffusely, resulting in low glitter. Filaments of the present invention exhibit good soil hiding and covering ability without sacrificing crush resistance and without increasing the volume of the polymer material in the fiber. The invention allows the use of less polymeric material, since the void content is higher than in conventional hollow filaments. This results in less material to be processed, disposed of and/or recycled. Such filaments are very suitable for carpets and other textile products which are desired to exhibit high cover, good soiling and durability performance, and natural glitter-free lusters. When used in apparel fabrics, the filaments of the invention provide good heat insulation.

Those skilled in the art, having the teachings of the present invention as hereinbefore set forth may effect numerous modifications thereto. It should be appreciated that such modifications are to be construed within the contemplation of the present invention, as defined by the appended claims.

## Claims

1. A thermoplastic filament (10) having a central axis (10A) therethrough, the filament (10) comprising:
a core portion (12) having N lobes (14) joined thereto, each lobe (14) having a tip (16) thereon, each lobe (14) being joined to the core portion (12) along an inscribing circle (22), each lobe (14) having at least one opening (40) therein, and the opening (40) in each lobe (14) being disposed between the tip (16) of the lobe (14) and the inscribing circle (22)
**characterized in that**
the core portion (12) has N stiffening ribs (30) formed therein, the ribs (30) extending radially inwardly toward the axis (10A) of the filament (10), the ribs (30) cooperating to define at least N hollow regions (36) in the core portion (12), each hollow region (36) aligning radially with a respective lobe (14), the opening (40) in each lobe (14) and the hollow region (36) of the core portion (12) corresponding to that lobe (14) cooperating to define a transverse stiffening web (42) extending across the lobe (14).

2. The filament (10) of claim 1, wherein each stiffening rib (30) has a radially inner end (32) thereon, the radially inner ends (32) of the ribs (30) being spaced from each other and from the central axis (10A) of the filament (10) thereby to define passages (46) within the core portion (12) through which the hollow regions (36) communicate with each other.

3. The filament (10) of claim 1, wherein each stiffening rib (30) is connected to the other of the ribs (30) along the axis (10A) of the filament (10), whereby the hollow regions (36) are isolated from each other.

4. The filament (10) of any one of claims 1 to 3, wherein each lobe (14) has at least a second opening (41) therein, the second opening (41) in each lobe (14) being disposed between the first opening (40) and the tip (16) of the lobe (14),
the first (40) and the second openings (41) in each lobe (14) cooperating to define a second transverse web (43) extending across the lobe (14).

5. The filament (10) of any one of claims 1 to 4, wherein each lobe (14) has a first (24A) and a second lateral edge (24B), the major portion of each lateral edge (24A; 24B) being substantially linear over substantially its entire length.

6. The filament (10) of any one of claims 1 to 4, wherein each lobe (14) has a first (24A) and a second lateral edge (24B), the major portion of each lateral edge (24A; 24B) is convexly curved over substantially its entire length.

7. A spinneret plate (50) for producing a thermoplastic synthetic polymer filament (10) according to any one of claims 1 to 6, wherein the spinneret plate (50). comprises a cluster of N peripheral slots (56) centered about a central point (58), each peripheral slot (56) comprising a pair of slot segments (60; 62) joined at a junction point (64), each slot segment (60; 62) in one peripheral slot (56) being confrontationally disposed with a slot segment in another peripheral slot, a rib-forming slot (66) extending from each junction point (64) toward the central point (58) of the cluster, at least one web-forming slot (70; 72) extending from each slot segment (60; 62) toward the slot segment with which it is confrontationally disposed.

8. The spinneret plate (50) of claim 7 further comprising a second web-forming slot (71; 73) extending from each slot segment (60; 62) toward the slot segment with which it is confrontationally disposed.

9. The spinneret plate (50) of any one of claims 7 and 8, wherein each rib-forming slot (66) extends at least two-thirds of the distance between the junction point (64) and the central point (58) of the cluster.

10. The spinneret plate (50) of any one of claims 7 and 8, wherein each rib-forming slot (66) extends less than one-half of the distance between the junction point (64) and the central point (58) of the cluster.

11. The spinneret plate (50) of any one of claims 7 to 10, wherein there are three pairs or four pairs of peripheral slot segments (56).

12. The spinneret plate (50) of any one of claims 7 to 11, wherein each peripheral slot segment (56) is substantially linear over substantially its entire length.

13. The spinneret plate (50) of any one of claims 7 to 11, wherein each peripheral slot segment (56) is convexly curved over substantially its entire length.

14. A carpet yarn having at least one thermoplastic filament (10) according to any one of claims 1 to 6.

15. The use of a yam according to claim 14 for the manufacture of a carpet.

## Patentansprüche

1. Thermoplastischer Faden (10) mit einer durch denselben verlaufenden zentralen Achse (10A), wobei der Faden folgende Merkmale aufweist:
einen Kernbereich (12) mit N Profilvorsprüngen (14), die mit demselben verbunden sind, wobei jeder Profilvorsprung (14) eine Spitze (16) aufweist, wobei jeder Profilvorsprung (14) entlang einem einbeschriebenen Kreis (22) mit dem Kembereich (12) verbunden ist, wobei jeder Profilvorsprung (14) zumindest eine Öffnung (40) aufweist und die Öffnung (40) in jedem Profilvorsprung (14) zwischen der Spitze (16) des Profilvorsprungs (14) und dem einbeschriebenen Kreis (22) angeordnet ist.
**dadurch gekennzeichnet, daß**
im Kembereich (12) N Versteifungsrippen (30) ausgebildet sind, wobei sich die Rippen (30) zur Achse (10A) des Fadens (10) radial nach innen hin erstrecken, wobei die Rippen (30) zusammenwirken, um zumindest N Hohlbereiche (36) im Kembereich (12) zu definieren, wobei jeder Hohlbereich (36) radial mit einem jeweiligen Profilvorsprung (14) ausgerichtet ist, wobei die Öffnung (40) in jedem Profilvorsprung (14) und der Hohlbereich (36) des Kembereichs (12), der mit diesem Profilvorsprung (14) korrspondiert, zusammenwirken, um ein querverlaufendes Versteifungsgewebe (42) zu definieren, das sich über den Profilvorsprung (14) erstreckt.

2. Faden (10) nach Anspruch 1, bei dem jede Versteifungsrippe (30) ein radial inneres Ende (32) aufweist, wobei die radial inneren Enden (32) der Rippen (30) voneinander und von der zentralen Achse (10A) des Fadens (10) beabstandet sind, um dadurch Durchlässe (46) im Kembereich (12) zu definieren, durch welche die Hohlbereiche (36) miteinander kommunizieren.

3. Faden (10) nach Anspruch 1, bei dem jede Versteifungsrippe (30) mit den anderen Rippen (30) entlang der Achse (10A) des Fadens (10) verbunden ist, wodurch die Hohlbereiche (36) voneinander isoliert sind.

4. Faden (10) nach einem der Ansprüche 1 bis 3, bei dem jeder Profilvorsprung (14) zumindest eine zweite Öffnung (41) aufweist, wobei die zweite Öffnung (41) in jedem Profilvorsprung (14) zwischen der ersten Öffnung (40) und der Spitze (16) des Profilvorsprungs (14) angeordnet ist,
wobei die erste (40) und die zweite Öffnung (41) in jedem Profilvorsprung (14) zusammenwirken, um ein zweites querverlaufendes Gewebe (43) zu definieren, das sich über den Profilvorsprung (14) erstreckt.

5. Faden (10) nach einem der Ansprüche 1 bis 4, bei dem jeder Profilvorsprung (14) eine ersten (24A) und einen zweiten (24B) Seitenrand aufweist, wobei der Hauptabschnitt eines jeden Seitenrands (24A; 24B) im wesentlichen linear über im wesentlichen seine gesamte Länge verläuft.

6. Faden (10) nach einem der Ansprüche 1 bis 4, bei dem jeder Profilvorsprung (14) einen ersten (24A) und einen zweiten (24B) Seitenrand aufweist, wobei der Hauptabschnitt eines jeden Seitenrands (24A; 24B) im wesentlichen über seine gesamte Länge konvex gekrümmt ist.

7. Spinndüsenplatte (50) zur Herstellung eines thermoplastischen synthetischen Polymerfadens (10) nach einem der Ansprüche 1 bis 6, wobei die Spinndüsenplatte (50) eine Gruppierung von N peripheren Schlitzen (56) aufweist, die um einen Mittelpunkt (58) zentriert angeordnet sind, wobei jeder periphere Schlitz (56) ein Paar von Schlitzsegmenten (60; 62) aufweist, die an einem Verbindungspunkt (64) zusammenlaufen, wobei jedes Schlitzsegment (60; 62) in einem peripheren Schlitz (56) gegenüber einem Schlitzsegment in einem anderen peripheren Schlitz (56) angeordnet ist, wobei sich ein rippenbildender Schlitz (66) von jedem Verbindungspunkt (64) zum Mittelpunkt (58) der Gruppierung hin erstreckt, wobei sich zumindest ein gewebebildender Schlitz (70; 72) von jedem Schlitzsegment (60; 62) zu dem Schlitzsegment hin erstreckt, gegenüber dem er angeordnet ist.

8. Spinndüsenplatte (50) nach Anspruch 7, die ferner einen zweiten gewebebildenden Schlitz (71; 73) aufweist, der sich von jedem Schlitzsegment (60; 62) zu dem Schlitzsegment hin erstreckt, gegenüber dem er angeordnet ist.

9. Spinndüsenplatte (50) nach Anspruch 7 oder 8, bei der sich jeder rippenbildende Schlitz (66) über zumindest zwei Drittel der Entfernung zwischen dem Verbindungspunkt (64) und dem Mittelpunkt (58) der Gruppierung erstreckt.

10. Spinndüsenplatte (50) nach Anspruch 7 oder 8, bei der sich jeder rippenbildende Schlitz (66) über weniger als die Hälfte der Entfernung zwischen dem Verbindungspunkt (64) und dem Mittelpunkt (58) der Gruppierung erstreckt.

11. Spinndüsenplatte (50) nach einem der Ansprüche 7 bis 10, bei der drei oder vier Paare von peripheren Schlitzsegmenten (56) vorliegen.

12. Spinndüsenplatte (50) nach einem der Ansprüche 7 bis 11, bei der jedes periphere Schlitzsegment (56) über im wesentlichen seine gesamte Länge im wesentlichen linear verläuft.

13. Spinndüsenplatte (50) nach einem der Ansprüche 7 bis 11, bei der jedes periphere Schlitzsegment (56) über im wesentlichen seine gesamte Länge konvex gekrümmt ist.

14. Teppichgam mit zumindest einem thermoplastischen Faden (10) nach einem der Ansprüche 1 bis 6.

15. Verwendung eines Garns nach Anspruch 14 für die Herstellung eines Teppichs.

## Revendications

1. Filament thermoplastique (10) possédant un axe central (10A) à travers celui-ci, le filament (10) comprenant:
une partie centrale (12) possédant N lobes (14) joints à celle-ci, chaque lobe (14) présentant une extrémité (16) sur celui-ci, chaque lobe (14) étant joint à la partie centrale (12) le long d'un cercle inscrit (22), chaque lobe (14) présentant au moins une ouverture (40) dans celui-ci, et l'ouverture (40) dans chaque lobe (14) étant disposée entre l'extrémité (16) du lobe (14) et le cercle inscrit (22),
**caractérisé en ce que**
la partie centrale (12) possède N nervures de raidissement (30) formées dans celle-ci, les nervures (30) s'étendant radialement vers l'intérieur vers l'axe (10A) du filament (10), les nervures (30) coopérant pour définir au moins N régions creuses (36) dans la partie centrale (12), chaque région creuse (36) s'alignant radialement avec un lobe respectif (14), l'ouverture (40) dans chaque lobe (14) et la région creuse (36) de la partie centrale (12) correspondant à ce lobe (14) coopérant pour définir une bande de raidissement transversale (42) s'étendant en travers du lobe (14).

2. Filament (10) suivant la revendication 1, dans lequel chaque nervure de raidissement (30) présente une extrémité radialement interne (32) sur celle-ci, les extrémités radialement internes (32) des nervures (30) étant espacées les unes des autres et de l'axe central (10A) du filament (10) pour définir de cette manière des passages (46) dans la partie centrale (12) par lesquels les régions creuses (36) communiquent les unes avec les autres.

3. Filament (10) suivant la revendication 1, dans lequel chaque nervure de raidissement (30) est reliée à l'autre des nervures (30) le long de l'axe (10A) du filament (10), en conséquence de quoi les régions creuses (36) sont isolées les unes des autres.

4. Filament (10) suivant l'une quelconque des revendications 1 à 3, dans lequel chaque lobe (14) présente au moins une deuxième ouverture (41) dans celui-ci, la deuxième ouverture (41) dans chaque lobe (14) étant disposée entre la première ouverture (40) et l'extrémité (16) du lobe (14), la première ouverture (40) et la deuxième ouverture (41) dans chaque lobe (14) coopérant pour définir une deuxième bande transversale (43) s'étendant en travers du lobe (14).

5. Filament (10) suivant l'une quelconque des revendications 1 à 4, dans lequel chaque lobe (14) présente un premier bord latéral (24A) et un deuxième bord latéral (24B), la majeure partie de chaque bord latéral (24A; 24B) étant substantiellement linéaire sur substantiellement sa longueur entière.

6. Filament (10) suivant l'une quelconque des revendications 1 à 4, dans lequel chaque lobe (14) présente un premier bord latéral (24A) et un deuxième bord latéral (24B), la majeure partie de chaque bord latéral (24A; 24B) étant courbée de façon convexe sur substantiellement sa longueur entière.

7. Plaque de filière (50) pour la production d'un filament polymère synthétique thermoplastique (10) suivant l'une quelconque des revendications 1 à 6, dans laquelle la plaque de filière (50) comprend un groupe de N fentes périphériques (56) centrées autour d'un point central (58), chaque fente périphérique (56) comprenant une paire de segments de fente (60; 62) joints à un point de jonction (64), chaque segment de fente (60; 62) dans une fente périphérique (56) étant disposé de manière à faire face à un segment de fente dans une autre fente périphérique, une fente formant une nervure (66) s'étendant à partir de chaque point de jonction (64) vers le point central (58) du groupe, au moins une fente formant une bande (70;72) s'étendant à partir de chaque segment de fente (60; 62) vers le segment de fente avec lequel il est disposé en lui faisant face.

8. Plaque de filière (50) suivant la revendication 7, comprenant en outre une deuxième fente formant une bande (71; 73) s'étendant à partir de chaque segment de fente (60; 62) vers le segment de fente avec lequel il est disposé en lui faisant face.

9. Plaque de filière (50) suivant l'une quelconque des revendications 7 et 8, dans laquelle chaque fente formant une nervure (66) s'étend au moins à deux tiers de la distance entre le point de jonction (64) et le point central (58) du groupe.

10. Plaque de filière (50) suivant l'une quelconque des revendications 7 et 8, dans laquelle chaque fente formant une nervure (66) s'étend à moins de la moitié de la distance entre le point de jonction (64) et le point central (58) du groupe.

11. Plaque de filière (50) suivant l'une quelconque des revendications 7 à 10, dans laquelle il y a trois paires ou quatre paires de segments de fente périphérique (56).

12. Plaque de filière (50) suivant l'une quelconque des revendications 7 à 11, dans laquelle chaque segment de fente périphérique (56) est substantiellement linéaire sur substantiellement sa longueur entière.

13. Plaque de filière (50) suivant l'une quelconque des revendications 7 à 11, dans laquelle chaque segment de fente périphérique (56) est courbé de manière convexe sur substantiellement sa longueur entière.

14. Fil de tapis possédant au moins un filament thermoplastique (10) suivant l'une quelconque des revendications 1 à 6.

15. Utilisation d'un fil suivant la revendication 14 pour la fabrication d'un tapis.
